

## 1

3,368,944

 X-RAY-CONTRAST MEDIUM WITH  
A DENSITY OF 0.8-1.1

Stig Jöhs Gustav Sandmark, Knut Wicksells Vag 19,  
Lund, Sweden, and Ernst Helmer Hagstam, Tuborgsgatan 1B, Malmö, Sweden

No Drawing. Continuation-in-part of application Ser. No. 251,760, Jan. 16, 1963. This application Feb. 9, 1965, Ser. No. 431,428

Claims priority, application Sweden, Jan. 23, 1962,  
723/62

7 Claims. (Cl. 167—95)

This application is a continuation-in-part of our application Ser. No. 251,760, filed Jan. 16, 1963, now abandoned.

In X-ray examination of the gastro-intestinal tract it is already known to use a contrast medium, a so-called radiopaque meal, which is swallowed by the patient. The X-ray contrast media generally used consist of e.g. a porridge or the like into which some substances with high X-ray absorbing capacity such as barium sulphate, bismuth subcarbonate, thorium oxide or an iodine-containing compound, have been stirred. However, these contrast media are far from perfect and cause undesired effects as they are of high density because of the addition of the heavy X-ray absorber.

The abdominal cavity is filled mainly with mobile organs of about the same density as water and usually the density of these mobile organs is about 1.03 to 1.06 g./cm.<sup>3</sup>. The contents of the gastro-intestinal tract are also of about the same density. Pressure measurements have shown that the abdominal cavity behaves like a closed cavity filled with water. Thus, with normal gastro-intestinal contents the hydrostatic pressure acting on the inside and the outside of a given segment of the intestinal wall is about the same.

The contrast media hitherto used for the X-ray examinations of the gastro-intestinal tract are of high density (about 1.4 to 2.0 g./cm.<sup>3</sup>) and therefore the hydrostatic pressure within the gastro-intestinal tract when being filled with such a contrast medium is higher than the hydrostatic pressure within the abdominal cavity but outside the gastro-intestinal tract. This difference in pressure distorts the gastro-intestinal tract with the result that the contrast medium cannot readily pass through the gastro-intestinal tract and possibly does not reach the parts of the stomach or intestine to be examined because the X-ray contrast medium sinks to those parts of the gastro-intestinal tract which happen to be lowermost at the time of the examination. This disadvantageous effect may cause difficulties in examinations for e.g. hiatus hernia.

Thus there is a need for an X-ray contrast medium of about the same density as that of the abdominal organs so that the X-ray contrast medium can pass through the gastro-intestinal tract like ordinary food in a physiologically correct way and independently of the patient's posture. Hitherto it has, however, not been possible to produce such contrast media and as far as we know prior-art contrast media all are of a density of at least 1.4 g./cm.<sup>3</sup>, which density cannot be reduced by known methods.

An object of the invention is to provide an X-ray contrast medium having such a density that it can pass through the gastro-intestinal tract like ordinary food in a physiologically correct way and independently of the patient's posture.

Another object of the invention is to provide an X-ray contrast medium having a density of 0.8 to 1.1 g./cm.<sup>3</sup>.

Still another object of the invention is to provide an X-ray contrast medium consisting of an X-ray absorber, a particulate resin foam, water and a thickening agent,

## 2

the proportions of said components being such that the X-ray contrast medium has a density of 0.8 to 1.1 g./cm.<sup>3</sup>.

A further object of the invention is to provide an X-ray contrast medium comprising a particulate, therapeutically acceptable resin foam, iodine chemically bonded to said resin foam, water and a non-toxic thickening agent, the proportions of said components being such that the X-ray contrast medium has a density of 0.8 to 1.1 g./cm.<sup>3</sup>.

According to the invention, the X-ray contrast medium comprises an X-ray absorber comprising a member of the group consisting of barium sulphate, bismuth subcarbonate, thorium oxide and iodine, a particulate, therapeutically acceptable resin foam comprising a member of the group consisting of polystyrenes, polyethylenes and urea resins, water and a non-toxic thickening agent of the group consisting of thickeners of seaweed origin, vegetable gums and water soluble cellulose esters, the proportions of said components being such that the X-ray contrast medium has a density of 0.8 to 1.1 g./cm.<sup>3</sup>.

The X-ray absorber is preferably homogeneously incorporated in the resin foam and in this case it is possible to prevent the X-ray absorber from coming in direct contact with the contents of the gastro-intestinal tract. Thus, as an X-ray absorber one may use an element or a compound that is toxic per se.

The X-ray contrast medium according to the invention may be prepared by preparing a thixotropic suspension of the X-ray absorber, e.g. barium sulphate, water, a suitable amount of a carrier material comprising particulate therapeutically acceptable resin foam and a non-toxic thickening agent, the relative amounts of the said components being such that the final X-ray contrast medium has a density of 0.8 to 1.1 g./cm.<sup>3</sup>.

Another possibility of preparing the X-ray contrast medium according to the invention is to melt the resin and incorporate the X-ray absorber by mixing it with the molten resin. The mixture may then be treated with air or gas, whereupon the mixture is allowed to set. The set material is ground and sieved to the desired particle size. The particles are then expanded in a well known way by heating them for a short period to about 90° C. so that the resin softens and the enclosed air or gas expands. Instead of melting the resin it is also possible to prepare a solution of the resin in a suitable solvent e.g. ethyl acetate and to suspend the X-ray absorber in the solution. Next, the suspension is spread in a thin layer and dried and then the dried material obtained is ground and sieved to the desired particle size. The particles are placed in a suitable fluid such as petroleum ether or pentane, for a period of e.g. 12 hours. During this time the particles swell. Excess fluid is then sucked off and the swollen particles are stirred in water at 90° C., thereby expanding.

The expanded particles prepared in either of the two above mentioned methods from a molten mass or a solution of the thermoplastic resin material, contain the bulk of the X-ray absorber within the particles. Any X-ray absorber on the surface of the particles can be washed off by artificial gastro-intestinal juice so that all X-ray absorber substance is contained within the resin particles and withdrawn from the gastro-intestinal juices in the patient's stomach and intestines. Thus, when using these methods of preparing the X-ray contrast medium it is possible to use X-ray absorbers which because of their toxicity could not hitherto with safety be considered as components of X-ray contrast media. Thus the invention has made it possible to use bismuth subcarbonate and thorium oxide as X-ray absorbers in X-ray contrast media for X-ray examination of the gastro-intestinal tract.

Still another possibility of preparing the X-ray con-

trast medium according to the invention is to prepare a solution of a volatile liquid and a film forming substance insoluble in the stomach comprising a member of the group consisting of shellac and cellulose acetate phthalate and to suspend the X-ray absorber in the solution. The foamed resin particles are then coated with the resultant mixture and the volatile liquid driven off. Any X-ray absorber not contained in and covered by the coating is removed e.g. by washing with artificial gastric juice. The coated particles are then suspended in a gel of water and a thickening agent in such a quantity that the final X-ray contrast medium has a density of 0.8 to 1.1 g./cm.<sup>3</sup>. This X-ray contrast medium is especially suitable in the X-ray examination of the ventricle and esophagus.

When iodine is used as the X-ray absorber it is possible to incorporate the absorber with the particulate resin foam by modifying the starting monomer from which the resin is prepared. In this case the iodine is chemically bonded to the monomer in a first stage and then the monomer is polymerized in well known manner. This modified iodine containing resin in a third stage is expanded in a manner well known in the art to produce particulate modified resin foam which is mixed with water and the non-toxic thickening agent, the proportions of the particulate modified resin foam, the water and the thickening agent being such that the final X-ray contrast medium has a density of 0.8 to 1.1 g./cm.<sup>3</sup>.

As the particulate resin foam in the X-ray contrast medium of the invention it is possible to use a polystyrene, polyethylene and urea resin. However, the preferred resins are the polystyrenes. All these resins can be prepared by methods well known in the art.

As a non-toxic thickening agent for use in the X-ray contrast medium of the invention it is possible to use vegetable gums, water, soluble cellulose esters and thickeners of seaweed origin e.g. alginates, agars and carageens.

Specific examples of thickening agents that have been used in X-ray contrast media of the invention are sodium alginate, potassium alginate, propylene glycol alginate, ammonium alginate, agar-agar, sodium carrageenate, potassium carrageenate, gum acacia, gum guar, gum locust, gum tragacanth, sodium carboxyl methyl cellulose, ethyl hydroxy ethyl cellulose and methyl cellulose.

The following examples will serve to illustrate the invention without limiting the same. In these examples all percentages and ratios refer to percentages and ratios by weight.

#### Example 1

Foamed polystyrene particles prepared in a known manner and having a diameter of about 0.5 mm. and a bulk density of about 0.1 to 0.2 g./cm.<sup>3</sup> were stirred into a 1% sodium alginate solution in water to provide them with a coating of sodium alginate. The particles were then removed from the sodium alginate solution and washed with water. Thereafter, the coated particles were suspended in a 0.1 N calcium chloride solution in water. Excess calcium chloride solution was allowed to drain off. In the meantime, barium sulphate (grade U.S.P.) had been suspended in the remainder of the original sodium alginate solution, and into this suspension the coated particles treated with calcium chloride were suspended. The calcium ions act as a stabilizer for the sodium alginate coating of the polystyrene particles and thus prevent the suspended barium sulphate and polystyrene particles from separating too rapidly when the X-ray contrast medium passes through the gastro-intestinal tract. The relative amounts of the ingredients were chosen in such a way that the final X-ray contrast medium had a bulk density of about 0.95 to 1.05 g./cm.<sup>3</sup>. Since the density of the X-ray contrast medium was about the same as that of the organs in the abdominal cavity the X-ray contrast medium could pass rapidly through

the stomach, the small intestine and large intestine in a physiologically correct way without it being necessary for the patient to be in a recumbent position and without any extraneous influence by pressure or turning of the patient. The X-ray contrast medium spread successively and in a thin even layer over the inner surfaces of the organs.

#### Example 2

The preparation of the X-ray contrast medium was carried out as described in Example 1 except that foamed polyethylene particles with a diameter of about 0.5 mm. and ammonium alginate were used instead of the polystyrene particles and the sodium alginate, respectively. The resulting X-ray contrast medium was found to act in a physiologically correct way when passing through the stomach, the small intestine and the large intestine, whereby the barium sulphate suspension spread successively and was distributed in a thin even layer over the inner surfaces of the organs.

#### Example 3

A 10 to 15% alcoholic solution of shellac or cellulose acetate phthalate was prepared. In this solution barium sulphate was suspended. Spherical foamed polystyrene particles having a diameter of about 0.1 mm. and prepared in a manner well known in the art were added to the suspension under stirring in such a quantity that the ratio of polystyrene particles to barium sulphate was about 1:2.5 by weight. The formation of large conglomerates of particles was prevented by means of talc or colloidal silica. Thereafter the material was dried and sieved and any unabsorbed barium sulphate was removed. The polystyrene particles thus coated with barium sulphate incorporated in a shellac or cellulose acetate phthalate layer were suspended in a 1% solution of ethyl hydroxy ethyl cellulose in water in such a quantity, that the final X-ray contrast medium had a density of about 0.8 to 1.1 g./cm.<sup>3</sup>. The X-ray contrast medium prepared in this way was found to be an excellent X-ray contrast medium for the X-ray examination of the gastro-intestinal tract.

#### Example 4

Example 3 was repeated except that thorium oxide was substituted for the barium sulfate and that gum tragacanth was substituted for the ethyl hydroxy ethyl cellulose. The final X-ray contrast medium having a density of about 0.8 to 1.1 g./cm.<sup>3</sup> was found to be an excellent X-ray contrast medium in the X-ray examination of the gastro-intestinal tract.

#### Example 5

100 g. polystyrene were dissolved in 300 ml. ethyl acetate. The solution was filtered and 200 g. bismuth subcarbonate were stirred into the filtrate. The solution was homogenized and spread in a thin layer on a polyethylene foil, where it was allowed to dry. After drying the material was ground in a mill with rotating knives until the material passed through a 50 mesh sieve (U.S. standard sieve). The powder was covered with petroleum ether and was allowed to stand for about 12 hours during which it was occasionally stirred. Afterwards excess petroleum ether was sucked off and the powder was sieved through a coarse sieve into water having a temperature of about 90° C. and in which the powder was vigorously stirred. The powder particles were thereby expanded and then they were immediately removed from the hot water, rinsed in cold water, dried and aired for some days. 50 g. of this material were stirred in about 100 ml. of a 1% solution of sodium carrageenate in water. The material thus prepared was an excellent X-ray contrast medium in X-ray examination of the gastro-intestinal tract.

#### Example 6

Example 5 was repeated except that thorium oxide was substituted for the bismuth subcarbonate. The final

suspension was found to be an excellent X-ray contrast medium in X-ray examination of the gastrointestinal tract.

*Example 7*

100 g. of a mixture of ortho and para iodine styrene monomer were polymerized in some well known manner e.g. through storing the monomer at 60° C. for a few hours with a small quantity of benzoylperoxide added. The obtained product containing 55% iodine was crushed into small particles and expanded as described in Example 5. The expanded iodine-containing resin particles were stirred into a 1% solution of methyl cellulose in water in such a quantity that the final product had a density of 0.95 to 1.05 g./cm.<sup>3</sup>. This product could be used as an X-ray contrast medium in X-ray examination of the gastro-intestinal tract.

*Example 8*

100 g. barium sulphate were thoroughly mixed into 50 g. of a urea resin premix. A curing agent solution was added and the mixture was whipped to obtain a foam with small homogeneous cells. After curing the product was ground and sieved and the fraction with a particle size between 0.1 and 0.5 mm. was used. This fraction was mixed with a 1% solution of potassium carrageenate in water in such a quantity that the final X-ray contrast medium had a density of 0.8 to 1.1 g./cm.<sup>3</sup>. This X-ray contrast medium was suitable for use in X-ray examination of the gastro-intestinal tract.

*Example 9*

100 g. polyethylene granules prepared in a known manner and containing an incorporated organic blowing agent were mixed with 100 g. barium sulphate. This material was extruded in thin sheets which during the extrusion expanded to a cellular product. This product was comminuted into particles about 0.5 mm. in diameter and was used in preparing an X-ray contrast medium by stirring the particles into an agar-agar gel in such a quantity that the final X-ray contrast medium had a density of about 0.95 to 1.05 g./cm.<sup>3</sup>. This X-ray contrast medium was suitable for use in X-ray examination of the gastro-intestinal tract.

The foregoing detailed description has been given for the purposes of illustration only and is not intended to limit the scope of the present invention which is to be determined from the appendant claims.

What we claim and desire to secure by Letters Patent is:

1. An X-ray contrast medium comprising an X-ray absorber comprising a member of the group consisting of barium sulphate, bismuth subcarbonate, thorium oxide and iodine, a particulate, therapeutically acceptable resin foam comprising a member of the group consisting of polystyrenes, polyethylenes and urea resins, water, and at most 1% based on the X-ray contrast medium of a non-toxic thickening agent of the group consisting of thickeners of seaweed origin, vegetable gums and water soluble cellulose esters, the proportions of said components being such that the X-ray contrast medium has a density of 0.8 to 1.1 g./cm.<sup>3</sup>.

2. The X-ray contrast medium according to claim 1, in which the proportions of said components are such that the X-ray contrast medium has a density of 0.95 to 1.05 g./cm.<sup>3</sup>.

3. An X-ray contrast medium comprising a particulate, therapeutically acceptable resin foam comprising a member of the group consisting of polystyrenes, polyethylenes and urea resins, an X-ray absorber comprising a member 5 of the group consisting of barium sulphate, bismuth subcarbonate, thorium oxide and iodine, said X-ray absorber being homogeneously incorporated in said particulate resin foam, water and at most 1% based on the X-ray contrast medium of a non-toxic thickening agent 10 of the group consisting of thickeners of seaweed origin, vegetable gums and water soluble cellulose esters, the proportions of said components being such that the X-ray contrast medium has a density of 0.8 to 1.1 g./cm.<sup>3</sup>.

4. The X-ray contrast medium according to claim 3, 15 wherein said X-ray absorber is barium sulphate and said resin foam is a polystyrene.

5. An X-ray contrast medium comprising a particulate, therapeutically acceptable polystyrene resin foam, iodine chemically bonded to said resin, water and at most 1% 20 based on the X-ray contrast medium of a non-toxic thickening agent of the group consisting of thickeners of seaweed origin, vegetable gums and water soluble cellulose esters, the proportions of said components being such that the X-ray contrast medium has a density of 0.8 to 1.1 25 g./cm.<sup>3</sup>.

6. An X-ray contrast medium comprising an X-ray absorber comprising a member of the group consisting of barium sulphate, bismuth subcarbonate, and thorium oxide, a particulate, therapeutically acceptable resin foam 30 comprising a member of the group consisting of polystyrenes, polyethylenes and urea resins, said particulate resin foam being coated with said X-ray absorber, water and at most 1% based on the X-ray contrast medium of a non-toxic thickening agent of the group consisting of 35 thickeners of seaweed origin, vegetable gums and water soluble cellulose esters, the proportions of said components being such that the X-ray contrast medium has a density of 0.8 to 1.1 g./cm.<sup>3</sup>.

7. An X-ray contrast medium comprising a particulate, 40 therapeutically acceptable resin foam comprising a member of the group consisting of polystyrenes, polyethylenes and urea resins, an X-ray absorber comprising a member 45 of the group consisting of barium sulphate, bismuth subcarbonate, and thorium oxide, a film forming substance insoluble in the stomach comprising a member 50 of the group consisting of shellac and cellulose acetate phthalate, said film forming substance substantially covering each particle of said particulate resin foam and said X-ray absorber being distributed in and covered by said 55 film forming substance, water and at most 1% based on the X-ray contrast medium of a non-toxic thickening agent of the group consisting of thickeners of seaweed origin, vegetable gums and water soluble cellulose esters, the proportions of said components being such that the X-ray contrast medium has a density of 0.8 to 1.1 g./cm.<sup>3</sup>.

**References Cited**

**FOREIGN PATENTS**

- 60 657,979 10/1951 Great Britain ----- 167—95  
 ELBERT L. ROBERTS, *Primary Examiner*.  
 LEWIS GOTTS, *Examiner*.  
 65 R. L. HUFF, *Assistant Examiner*.